

## UNITED STATES PATENT OFFICE

2,647,839

WATER DISPLACING RUST PREVENTIVE  
COMPOSITIONS AND PROCESS OF  
COATING A BASE THEREWITHWilliam A. Zisman, Washington, D. C., and  
Hayward R. Baker, Mount Rainier, Md.No Drawing. Application September 16, 1949,  
Serial No. 116,202

15 Claims. (Cl. 106—14)

(Granted under Title 35, U. S. Code (1952),  
sec. 266)

1

This invention relates to water-displacing corrosion-inhibiting compositions.

The so-called water-displacing compositions heretofore known in the art have been at best, mere corrosion-preventative agents, since none has been capable of displacing a water film of any appreciable thickness from a surface to be treated. Of all of the commercially available products examined in connection with the research on this subject, the present inventors found none that would displace a water layer as great as 2 mm. thick from a steel test-plate, and only one that would produce even the slightest displacement of a 1 mm. film of water from such a plate. Moreover, the commercial products studied were all found to include non-volatile components in excessive amounts ranging from 18% to 55%, leaving residual films upon the surfaces under treatment which were inordinately thick. Moreover, since none of these products was compatible with commercial types of electrical insulation, they are entirely unsuited for uses in which electrical equipment is encountered.

Now, by virtue of the present invention, a relatively high degree of water-displacement is achieved, non-volatile components are maintained at a very low value, film thickness is greatly reduced, and practically any type of material, including electrical insulation, can be treated with complete satisfaction.

The more important requirements of true water-displacing corrosion-inhibiting compositions include a high equilibrium spreading pressure to assure their complete distribution over the surface to be treated; they must displace the water in contact with such a surface; they should remain completely effective for extended storage periods; their major portions should evaporate rapidly; they should leave a relatively thin protective film on the surface under treatment; their flash points should be reasonably high; they should not be toxic; and they should not adversely affect the surface to be treated.

As set forth in a copending application Serial Number 781,108 filed October 21, 1947, now abandoned, of which this application is a continuation-in-part, when a true water-displacing corrosion-inhibiting composition is applied to a film of water covering a surface to be treated, the composition spreads very rapidly over the water film and by virtue of its solubility characteristics, penetrates the film, contacts the surface to be treated, and becomes adsorbed on the surface as an oriented monomolecular hy-

2

drophobic film covering the entire area. Inasmuch as the water-displacing component evaporates rather quickly, only the corrosion-inhibiting ingredient will remain to constitute a protective film.

Whereas a number of liquid polar compounds display many of the necessary characteristics, in that they possess high equilibrium spreading pressures, penetrate a relatively thick layer of water, and become adsorbed by underlying surfaces of various types to form thin hydrophobic films, these compounds alone have failed to provide a complete answer to the problem because they evaporate rapidly, failing to produce a lasting protective film on the surface under treatment. Exploration of many classes of compounds including alcohols, ethers, glycol-ethers, ketones, acetoacetates, lactates, carbonates and oxalates, has failed to indicate an individual compound possessing all of the characteristics required for a water-displacing corrosion-inhibiting composition suited for general application.

An intensive study of the compounds of these classes in combination with compatible compounds of a complementary nature, has led to the discovery of highly satisfactory water-displacing corrosion-inhibiting compositions possessing all of the necessary requirements. It has been found that certain alcohols are eminently suited for use as the water-displacing component in conjunction with various corrosion-inhibiting components which are miscible therewith in proportions of from 0.1% to less than 10.0% by weight, which are substantially non-volatile, which are polar, which have boiling points exceeding 150° C., and which possess a water solubility not exceeding 3.0% by weight.

Aliphatic monohydric alcohols containing fewer than four carbon atoms to the molecule are substantially completely soluble in water and are therefore unsuitable for the purposes contemplated; moreover, the low flash points of these compounds (under 100° F.) would render their use hazardous for many purposes. On the other hand, those aliphatic monohydric alcohols containing more than eight carbon atoms per molecule approach complete insolubility in water, a property which is inconsistent with the essential function of penetrating the water film to establish contact with the surface to be preserved. Thus, the aliphatic monohydric alcohols and mixtures thereof containing from 4 to 8 carbon atoms per molecule are those with which this invention is primarily concerned, and within this group,

those containing from 4 to 6 carbon atoms per molecule are particularly effective. More specifically, butanols and their mixtures, and pentanols and their mixtures, have displayed excellent properties as the water-displacing component.

It may be noted that these alcohols containing from 4 to 6 carbon atoms per molecule have equilibrium spreading pressures ranging from 38 to 50 dynes per cm., boiling points from 108° to 195° C., flash points from 115° to 165° F., and melting points from -108° to 40° C., thus adapting them for use over a wide range of temperatures without the creation of undue fire hazards.

The preferred categories of alcohols have been found to be compatible and effective with a large and diversified number of corrosion-inhibitors of the polar type, which are substantially non-volatile at temperatures below 150° C. and non-corrosive and a water solubility not exceeding 3% by weight. Such inhibitors include: oleic acid, phenyl undecylic acid, phenyl stearic acid, xylyl stearic acid, xenyl stearic acid, dodecyl phenyl stearic acid, naphthenic acid, sorbitan monooleate, mannan monooleate, sorbitan dilaurate, sorbitan triricinoleate, diglycol laurate, diglycol ricinoleate, diethyleneglycol monolaurate, glyceryl monooleate, glyceryl dioleate, zinc phenyl undecanoate, zinc ethyl phenyl stearate, magnesium phenyl stearate, calcium xenyl stearate, sodium petroleum sulfonate, barium petroleum sulfonate, dodecyl ammonium laurate, cyclohexyl ammonium laurate, and dicyclohexyl ammonium laurate.

Inasmuch as the compositions must sometimes be stored over long periods of time without loss of stability, various antioxidants may be added in small quantities without adversely affecting the required properties of the compositions. Antioxidants which have been employed advantageously for this purpose include: 2, 6-ditertiarybutyl-4-methylphenol (PX441); 2, 4-dimethyl-6-tertiarybutylphenol (24M6B); n-butylaminophenol combined with a small addition of butylphenylenediamine (UOP4); and di-sec-butyl-p-phenylenediamine (UOP5).

For applications in which high values of equilibrium spreading pressures are not necessary to produce the required results, the cost of the material can be reduced by the use of suitable diluents. It has been found that aliphatic hydrocarbons of the Stoddard types for example, such as "Varsol No. 1," may be used for dilution of the polar solvent. Tests have shown that the addition of up to 50% of "Varsol No. 1," cumene, or isoctane, to butanol mixtures, reduces the equilibrium spreading pressure at 20° C. by only a small amount and in a substantially linear fashion. For example, the addition of 20% of any of these three diluents decreases the equilibrium spreading pressure of the butanol mixture by only 2.5 dynes per cm. From these tests it has been concluded that up to 50% dilution with such hydrocarbons is consistent with reasonably effective results, and even greater dilution with more polar liquids may be feasible, provided that the particular diluent selected is adequate from the standpoints of volatility and flash point, and more important, that it does not substantially reduce the water-displacing property of the composition.

It is among the objects of the present invention to produce a water-displacing corrosion-inhibiting composition comprising more than 90% by weight of an aliphatic monohydric alcohol or mix-

ture of aliphatic monohydric alcohols containing from 4 to 8 carbon atoms and a straight chain of at least 3 carbon atoms per molecule; and miscible proportions of from 0.1% to less than 10% by weight of a polar-type rust inhibitor which is substantially non-volatile at temperatures below 150° C. and has a water solubility not exceeding 3% by weight. The preferred alcohol or alcohol mixture will contain from 4 to 6 carbon atoms per molecule, particularly favorable results having been experienced with butanols and butanol mixtures having a boiling point between 100° and 120° C. and a flash point above 90° F., and pentanols and pentanol mixtures having a boiling point between 112° and 140° C. and a flash point above 100° F. Advantageous results have attended the inclusion of less than 1% by weight of an antioxidant, and diluents in proportions not exceeding 50% of the weight of the composition have been employed in some cases. Among the rust inhibitors producing desirable results, glyceryl oleates and dioleates have been highly satisfactory. A highly desirable characteristic of many of the compositions contemplated herein is their property of removing fingerprint acids from surfaces.

Specific aliphatic alcohols of the type mentioned which have been productive of good results, include 1 - butanol, 1 - pentanol, 3 - methyl - 1 - butanol, 2-methyl-1-butanol, 3-pentanol and 2-ethyl-1-butanol.

The water-displacing corrosion-inhibiting compositions contemplated herein are very useful for treating apparatus and equipment after exposure to seawater or fresh water, and find immediate application in connection with marine salvage operations. A specific example indicating suitable procedural steps utilizing the compositions of the present invention is outlined as follows:

An Allis-Chalmers motor-generator set, comprising a 115 volt D. C. motor, a 1-kw.-115 volt A. C. generator, and a Cutler-Hammer controller for the motor, was operated for forty-eight hours under a load of 1320 watts, during which a number of resistance values were observed. This equipment was then immersed in a tank of synthetic sea water for a period of one week, then removed and washed three times with city tap water. The equipment was then subjected to a compressed air blast for about ten minutes, and then sprayed by means of a conventional air spray gun with approximately one liter of a water-displacing corrosion-inhibiting composition comprising a technical grade of n-butyl alcohol and 0.5% by weight of a concentrate of a commercial mixture of glyceryl monooleate and glyceryl dioleate. Evaporation of the water and n-butyl alcohol was accelerated by applying a blast of air at a temperature of 200° F. using an electrical blower. This was continued for about thirty minutes, whereupon the various elements of the equipment were tested for electrical resistance and compared with the corresponding data obtained prior to immersion.

The resistance readings of the motor components compared as follows:

|                            | Ohms Before Immersion | Ohms After Immersion |
|----------------------------|-----------------------|----------------------|
| Shunt field.....           | 195.....              | 180.....             |
| Series field to frame..... | infinite.....         | 350.....             |
| Shunt field to frame.....  | do.....               | infinite.....        |
| Both fields to frame.....  | do.....               | 500.....             |

The resistance readings of the controller compared as follows:

|                                    | Ohms Before Immersion | Ohms After Immersion |
|------------------------------------|-----------------------|----------------------|
| Magnet winding to fixed resistance | 550                   | 400                  |
| Magnet winding                     | 58                    | 45                   |
| Line to variable resistance        | 550                   | 500                  |

After obtaining these readings, the motor was started at a low voltage which was gradually increased in order to warm the armature and fields and thereby expedite the evaporation of the water-butyl alcohol mixture. The voltage was increased to the normal rating in approximately one hour, and the set then ran under load for 48 hours, by which time the resistance values had increased to 90% of their original values before immersion.

The residual polar, monomolecular, hydrophobic rust inhibiting film remained on the surfaces for at least six months, at which time an inspection showed no evidence of corrosion, and no damage to insulation.

Typical examples of compositions contemplated by the present invention are listed below, the proportions being based upon weight, and the "Displacement" value being the number of millimeters a film of water 1 mm. thick is displaced by the deposition of a 0.025 ml. drop of the composition on the surface of the water.

*Example 1*

|                     |         |      |
|---------------------|---------|------|
| 1-pentanol          | percent | 98.9 |
| Glyceryl oleate     | do      | 1.0  |
| Antioxidant (PX441) | do      | 0.1  |
| Displacement        | mm      | 44.5 |

*Example 2*

The composition of Example 1 diluted with 15% "Varsol No. 1."

|              |    |      |
|--------------|----|------|
| Displacement | mm | 38.0 |
|--------------|----|------|

*Example 3*

|                 |         |      |
|-----------------|---------|------|
| 1-butanol       | percent | 98.9 |
| Glyceryl oleate | do      | 1.0  |
| Antioxidant     | do      | 0.1  |
| Displacement    | mm      | 50.5 |

*Example 4*

The composition of Example 3 diluted with 15% "Varsol No. 1."

|              |    |      |
|--------------|----|------|
| Displacement | mm | 38.5 |
|--------------|----|------|

*Example 5*

|                     |         |      |
|---------------------|---------|------|
| 3-methyl-1-butanol  | percent | 98.9 |
| Glyceryl oleate     | do      | 1.0  |
| Antioxidant (PX441) | do      | 0.1  |
| Displacement        | mm      | 44.0 |

*Example 6*

The composition of Example 5 diluted with 15% "Varsol No. 1."

|              |    |      |
|--------------|----|------|
| Displacement | mm | 37.5 |
|--------------|----|------|

*Example 7*

|                            |         |      |
|----------------------------|---------|------|
| 3-pentanol                 | percent | 98.9 |
| Sodium petroleum sulfonate | do      | 1.0  |
| Antioxidant (24M6B)        | do      | 0.1  |
| Displacement               | mm      | 45.0 |

*Example 8*

The composition of Example 7 diluted with 15% "Varsol No. 1."

|              |    |      |
|--------------|----|------|
| Displacement | mm | 38.5 |
|--------------|----|------|

*Example 9*

|                     |         |      |
|---------------------|---------|------|
| 2-methyl-1-butanol  | percent | 98.9 |
| Glyceryl oleate     | do      | 1.0  |
| Antioxidant (24M6B) | do      | 0.1  |
| Displacement        | mm      | 51.0 |

*Example 10*

The composition of Example 9 diluted with 15% "Varsol No. 1."

|              |    |      |
|--------------|----|------|
| Displacement | mm | 44.0 |
|--------------|----|------|

*Example 11*

The composition of Example 9 diluted with 30% "Varsol No. 1."

|              |    |      |
|--------------|----|------|
| Displacement | mm | 37.0 |
|--------------|----|------|

*Example 12*

|                     |         |      |
|---------------------|---------|------|
| 2-ethyl-1-butanol   | percent | 98.9 |
| Glyceryl oleate     | do      | 1.0  |
| Antioxidant (PX441) | do      | 0.1  |
| Displacement        | mm      | 50.5 |

*Example 13*

The composition of Example 12 diluted with 15% "Varsol No. 1."

|              |    |      |
|--------------|----|------|
| Displacement | mm | 43.5 |
|--------------|----|------|

*Example 14*

|                            |         |      |
|----------------------------|---------|------|
| Commercial mixed pentanols | percent | 98.9 |
| Glyceryl oleate            | do      | 1.0  |
| Antioxidant (PX441)        | do      | 0.1  |
| Displacement               | mm      | 43.0 |

*Example 15*

The composition of Example 14 diluted with 15% "Varsol No. 1."

|              |    |      |
|--------------|----|------|
| Displacement | mm | 37.0 |
|--------------|----|------|

*Example 16*

|                     |         |      |
|---------------------|---------|------|
| 1-butanol           | percent | 50.0 |
| 1-pentanol          | do      | 48.9 |
| Glyceryl oleate     | do      | 1.0  |
| Antioxidant (PX441) | do      | 0.1  |
| Displacement        | mm      | 46.0 |

*Example 17*

The composition of Example 16 diluted with 15% "Varsol No. 1."

|              |    |      |
|--------------|----|------|
| Displacement | mm | 39.0 |
|--------------|----|------|

*Example 18*

|                            |         |      |
|----------------------------|---------|------|
| 1-butanol                  | percent | 50.0 |
| 2-ethyl-1-butanol          | do      | 48.9 |
| Sodium petroleum sulfonate | do      | 1.0  |
| Antioxidant (PX441)        | do      | 0.1  |
| Displacement               | mm      | 45.5 |

*Example 19*

The composition of Example 18 diluted with 15% "Varsol No. 1."

|              |    |      |
|--------------|----|------|
| Displacement | mm | 38.0 |
|--------------|----|------|

*Example 20*

|                     |         |      |
|---------------------|---------|------|
| 1-butanol           | percent | 94.9 |
| Glyceryl oleate     | do      | 5.0  |
| Antioxidant (PX441) | do      | 0.1  |
| Displacement        | mm      | 50.0 |

*Example 21*

The composition of Example 20 diluted with 15% "Varsol No. 1."

|              |    |      |
|--------------|----|------|
| Displacement | mm | 38.0 |
|--------------|----|------|

## Example 22

The composition of Example 20 diluted with 30% "Varsol No. 1."

Displacement mm. 37.0

## Example 23

The composition of Example 20 diluted with 50% "Varsol No. 1."

Displacement mm. 35.0

## Example 24

1-butanol percent 90.0

Glyceryl oleate do 9.9

Antioxidant (PX441) do 0.1

Displacement mm. 48.5

## Example 25

The composition of Example 24 diluted with 15% "Varsol No. 1."

Displacement mm. 38.5

## Example 26

1-pentanol percent 98.9

Cyclohexylammoniumlaurate do 1.0

Antioxidant (PX441) do 0.1

Displacement mm. 44.5

## Example 27

The composition of Example 26 diluted with 15% "Varsol No. 1."

Displacement mm. 37.5

Inasmuch as there is a practical limit to the number of examples to be presented, and to the amount of detail to be recited, the foregoing material should be regarded in an illustrative sense, and not limiting beyond the scope of the appended claims.

The invention described herein may be manufactured and used by or for the Government of the United States of America for governmental purposes without the payment of any royalties thereon or therefor.

What is claimed is:

1. A water-displacing corrosion-inhibiting composition consisting essentially of more than 90% by weight of at least one aliphatic monohydric alcohol having from 4 to 8 carbon atoms and a straight chain of at least 3 carbon atoms and miscible proportions of from 0.1 to less than 10% by weight of a polar type rust inhibitor which has a water solubility not exceeding 3% by weight and is substantially non-volatile at temperatures below 150° C.

2. A water-displacing corrosion-inhibiting composition consisting essentially of more than 90% by weight of at least one aliphatic monohydric alcohol having from 4 to 6 carbon atoms and a straight chain of at least 3 carbon atoms and miscible proportions of from 0.1 to less than 10% by weight of a polar type rust inhibitor which has a water solubility not exceeding 3% by weight and is substantially non-volatile at temperatures below 150° C.

3. A water-displacing corrosion-inhibiting composition consisting essentially of more than 90% by weight of at least one aliphatic monohydric alcohol having from 4 to 8 carbon atoms and a straight chain of at least 3 carbon atoms, miscible proportions of from 0.1 to less than 10% by weight of a polar type rust inhibitor which has a water solubility not exceeding 3% by weight and is substantially non-volatile at temperatures

below 150° C., and less than 1% by weight of an antioxidant.

4. A water-displacing corrosion-inhibiting composition consisting essentially of more than 90% by weight of at least one aliphatic monohydric alcohol having from 4 to 8 carbon atoms and a straight chain of at least 3 carbon atoms, miscible proportions of from 0.1 to less than 10% by weight of a polar type rust inhibitor which has a water solubility not exceeding 3% by weight and is substantially non-volatile at temperatures below 150° C., and a liquid hydrocarbon diluent of the Stoddard type in proportions not exceeding 50% of the weight of said composition.

5. A water-displacing corrosion-inhibiting composition consisting essentially of more than 90% by weight of at least one aliphatic monohydric alcohol having from 4 to 8 carbon atoms and a straight chain of at least 3 carbon atoms, miscible proportions of from 0.1 to less than 10% by weight of a polar type rust inhibitor which has a water solubility not exceeding 3% by weight and is substantially non-volatile at temperatures below 150° C., less than 1% by weight of an antioxidant, and a liquid hydrocarbon diluent of the Stoddard type in proportions not exceeding 50% of the weight of said composition.

6. A water-displacing corrosion-inhibiting composition consisting essentially of more than 90% by weight of mixed butanols having a boiling point between 100 and 120° C. and a flash point above 90° F. and miscible proportions of from 0.1 to less than 10% by weight of a polar type rust inhibitor which has a water solubility not exceeding 3% by weight and is substantially non-volatile at temperatures below 150° C.

7. A water-displacing corrosion-inhibiting composition as set forth in claim 6 containing a liquid hydrocarbon diluent of the Stoddard type in proportions not exceeding 50% of the weight of said composition.

8. A water-displacing corrosion-inhibiting composition as set forth in claim 6 containing less than 1% by weight of an antioxidant.

9. A water-displacing corrosion-inhibiting composition as set forth in claim 8 containing a liquid hydrocarbon diluent of the Stoddard type in proportions not exceeding 50% of the weight of said composition.

10. A water-displacing corrosion-inhibiting composition consisting essentially of more than 90% by weight of at least one aliphatic monohydric alcohol having from 4 to 8 carbon atoms and a straight chain of at least 3 carbon atoms and 0.1 to less than 10% by weight of a glyceryl oleate.

11. A water-displacing corrosion-inhibiting composition consisting essentially of more than 90% by weight of mixed butanols having a boiling point between 100 and 120° C. and a flash point above 90° F. and from 0.1 to less than 10% by weight of a glyceryl oleate.

12. A water-displacing corrosion-inhibiting composition consisting essentially of more than 90% by weight of mixed pentanols having a boiling point between 112 and 140° C. and a flash point above 100° F. and from 0.1 to less than 10% by weight of a glyceryl oleate.

13. A method of displacing water from and inhibiting corrosion of a water-wet surface which comprises applying to said wet surface a composition comprising more than 90% by weight of at least one aliphatic monohydric alcohol having from 4 to 8 carbon atoms and a straight chain of at least 3 carbon atoms and miscible proportions

of from 0.1 to less than 10% by weight of a polar type rust inhibitor which has a water solubility not exceeding 3% by weight and is substantially non-volatile at temperatures below 150° C.

14. A method of displacing water from and inhibiting corrosion of a water-wet surface which comprises applying to said wet surface a composition comprising more than 90% by weight of at least one aliphatic monohydric alcohol having from 4 to 6 carbon atoms and a straight chain of at least 3 carbon atoms and miscible proportions of from 0.1 to less than 10% by weight of a polar type rust inhibitor which has a water solubility not exceeding 3% by weight and is substantially non-volatile at temperatures below 150° C.

15. A method of displacing water from and inhibiting corrosion of a water-wet surface which comprises applying to said wet surface a composition comprising more than 90% by weight of 1-

butanol and miscible proportions of from 0.1 to less than 10% by weight of a polar type rust inhibitor which has a water solubility not exceeding 3% by weight and is substantially non-volatile at temperatures below 150° C.

WILLIAM A. ZISMAN.  
HAYWARD R. BAKER.

References Cited in the file of this patent

UNITED STATES PATENTS

| Number    | Name                   | Date          |
|-----------|------------------------|---------------|
| 2,339,200 | Sowa -----             | Jan. 11. 1944 |
| 2,426,496 | Farley -----           | Aug. 26, 1947 |
| 2,481,372 | Von Fuchs et al. ----- | Sept. 6, 1949 |

OTHER REFERENCES

Handbook of Chemistry and Physics 28th Ed.  
1944, Chemical Rubber Publ. Co., pages 802-803.